

Mar. 27, 1923.

1,449,981.

E. T. GARSED.  
METHOD OF INDIGO DYEING.  
FILED AUG. 5, 1922.



Edward T. Garsed

By Church & Church

Attorneys

## UNITED STATES PATENT OFFICE.

EDWARD T. GARSED, OF CHARLOTTE, NORTH CAROLINA, ASSIGNOR TO ALEXANDER AND GARSED, INC., OF CHARLOTTE, NORTH CAROLINA, A CORPORATION OF NORTH CAROLINA.

## METHOD OF INDIGO DYEING.

Application filed August 5, 1922. Serial No. 579,793.

To all whom it may concern:

Be it known that I, EDWARD T. GARSED, a citizen of the United States, residing at Charlotte, in the county of Mecklenburg and 5 State of North Carolina, have invented certain new and useful Improvements in Methods of Indigo Dyeing; and I do hereby declare the following to be a full, clear, and exact description of the same, reference being had to the accompanying drawings, forming part of this specification.

This invention relates to the dyeing of yarn preparatory to weaving the yarn into cloth, and has for its object the provision 15 of a method of treating the yarn with greater convenience and more expedition while preserving all of the advantages of the present methods of dyeing.

It is customary at the present time to wind 20 yarn upon beams having a perforated or otherwise foraminous cylinder and to apply the coloring matter to the yarn on the beam by forcing dye liquor through the cylinder and out through the yarn, and then reversing 25 the process and forcing the liquor through the yarn and withdrawing it from the center of the cylinder, repeating these steps as many times as necessary, and it is also old to dye the yarn as single strands 30 and also as a sheet, but in each case the yarn is handled in a single manner throughout the process; that is, when the yarn is dyed on the beam it is oxidized on the beam by blowing compressed air through the cylinder, and when the rope or yarn is dyed in 35 strands or in a sheet the oxidizing of the indigo dye is obtained by passing the yarn as strands or in a sheet as the case may be through flutter rolls for exposure to the atmosphere for the appropriate time, and it is 40 new, so far as I am aware, to dye the yarn on the beam and then to oxidize the dye while the yarn is extended as a strand or as 45 a sheet, followed by a rewinding of the yarn on a beam similar to the original beam.

While I will describe my process in connection with the dyeing of blue denim, this is a mere illustrative example and it is my intention to use the process to dye other fibers such as silk, flax, and wool, and to make various other fabrics, such as ginghams, chambrays, etc. My process may be limited, however, to such dyes, for example,

indigo, as require oxidization to obtain the desired color, it being well known that an indigo dyed fabric is green when it comes from the bath and only obtains its blue color after exposure to the air. 55

In the drawings,—

Figure 1 is a diagrammatic elevation of a 60 dyeing machine;

Fig. 2 is a similar view of a rebeaming mechanism.

In carrying out this method, the yarn is first wound on the hollow beams 10, a number of which, preferably four, are then placed in the casings 11 of the dyeing machine, where the beams are held down against the dye inlets 12 by means of clamps 14. The hot water from the tank 15 is now 70 drawn past valve 16 and pipe 17 to the pump 18 and discharged via pipe 19 to the inlets 12 in communication with the perforated hollow cylinders of the beams. This boiling water passes through the yarn and falls 75 by gravity to the tank 20 which has an orifice 21 to which the suction pipe 17 is connected. When the boiling is completed the valve 16 is closed and the valve 25 is opened, thus connecting the indigo supply tank 26 with 80 the pump 18.

The indigo dye liquor is forced through the yarn in one way only, the so-called "inside-out" method, that is, the liquor is discharged by pipe 19 to the hollow center of 85 the beam and, passing through the foraminated or reticulate wall of the cylinder, dyes the yarn wound thereon. The length of time the dye is forced through the yarn depends entirely upon the mill. For my own part, I pass the dye liquor through the yarn for nearly an hour for each application of color, giving the yarn four separate applications for a dark blue denim of the standard overall color. 95

After the first application of color has been run as described the valve 25 may be closed and the valve 16 opened to wash the yarn again, but I almost invariably omit this washing at this time, although I sometimes wash the yarn in the dye machine just after the fourth or final application of the dye. From the dye machine the beams are taken to the rewinder shown in Fig. 2. My preference is to use four re-winders, one for 100 each beam and to run the re-winders at such 105

a speed that the time of re-winding after the final dyeing is approximately the same as the time required in the dyeing machine.

The once-dyed beam 10 is now placed on the stand 30 and the yarn directed over the flutter rolls 31, 32, etc., of the oxidizing frame to a power-driven winding mechanism 34 which should have a variable speed in order to drive the yarn at proper speed 5 for the different coats of dye, the yarn after the first application of dye requiring only about a minute to oxidize while requiring about two minutes after the third and approximately four minutes after the fourth 10 and final dye bath. The guide roll 36 and the adjustable leese comb 37 are of standard type and are used in the customary manner. It is to be noted that the end of the yarn that was on the outside of the beam 10 is on 15 the inside or cylinder side of the beam 10<sup>a</sup>, so that when the beam 10<sup>a</sup> is returned to the dyeing machine, that portion of the yarn which is of paler color, having previously been on the outside of the beam 10, is now 20 the first to be reached by the second batch of dye, so that, after the second forcing of dye through the yarn, the two ends of each warp yarn are of exactly the same shade. I may wash the yarn as it passes from the 25 last flutter roll 33 to the guide roll 36, although I prefer not to wash the yarn until after the final dye treatment in the machine, and during the last rewinding it is preferable to pass the yarn through a washer and 30 through a dryer, each of standard type, before it passes to the comb. When the yarn is wound on the beam 10<sup>a</sup> after the final dye bath, oxidization, washing and drying, it is 35 ready for the slasher. It is often convenient, however, to drive out the excess liquor 40 after each dyeing operation, before inserting the beam in the re-winder.

The principal advantage of the present method is the increased output possible.

45 When the yarn is dyed, washed and oxidized, in thread form, the dyeing must be regulated in accordance with the slowest part of the process, namely, the oxidizing. This requires the use of numbers of compensators, since the yarn must necessarily move at a constant rate through the dye. On the other hand, if the dyeing and oxidizing are both done while the yarn is wound on the beam, it is not possible to secure absolutely perfect color, since, for some unknown reason the use of compressed air dulls the color to an objectionable shade. To obtain a bright color,—one that is full of "bloom" 50—it seems essential to expose the fabric to air not under pressure. It is possible that the dulling of the color by compressed air is due to the moisture content of such air.

What I claim is:

1. The method of dyeing yarn which consists in winding the yarn on a beam, forcing

dye liquor through the yarn while on the beam, rebeaming the yarn, and in oxidizing the dye while rebeaming.

2. The method of dyeing yarn which consists in winding the yarn on a beam, forcing 70 dye liquor through the yarn while on the beam, washing the yarn while still on the beam, rebeaming the yarn, and in oxidizing the dye while rebeaming.

3. The method of dyeing yarn which consists in winding the yarn on a beam, forcing 75 dye liquor through the yarn while on the beam, rebeaming the yarn, and in oxidizing the dye, and washing and drying the yarn while rebeaming.

4. The method of dyeing yarn which consists in winding the yarn on a beam, forcing 80 dye liquor through the yarn while on the beam, washing the yarn while still on the beam, rebeaming the yarn, and in oxidizing 85 the dye and washing and drying the yarn while rebeaming.

5. The method of dyeing yarn which consists in winding the yarn on a beam, forcing 90 dye liquor through the yarn while on the beam, rebeaming the yarn, and in oxidizing the dye while rebeaming, forcing dye liquor through the yarn while on the second beam, rewinding the yarn, and in oxidizing the dye while the yarn is passing from the second beam to the final beam. 95

6. The method of dyeing yarn which consists in winding the yarn on a beam, forcing 100 dye liquor through the yarn while on the beam, rebeaming the yarn, oxidizing the dye while rebeaming, forcing dye liquor through the yarn while on the second beam, rewinding the yarn, and in oxidizing the dye while the yarn is being rebeamed.

7. The method of dyeing yarn with an 105 oxidizing color which consists in winding the yarn on a beam, applying color to the yarn while on said beam, rebeaming the yarn, and in oxidizing the dye while rebeaming.

8. The method of dyeing yarn which consists in winding the yarn on a support, applying color to the yarn while on said support, oxidizing said color and washing said 110 yarn while removing said yarn from said support.

9. The method of applying indigo color to yarn which consists in passing dye liquor through a hollow beam and the yarn thereon, oxidizing the dye while rewinding the yarn 115 on a beam with the formerly outside ends of the yarn now nearest the cylinder, forcing dye liquor through the second beam, repeating the above process until the desired color is secured, and finally drying the yarn. 120

10. The method of applying indigo color to cotton warp threads, which consists in winding said threads on a hollow support, discharging indigo liquor to the center of the support to pass through the threads, re- 125 130

versing the winding of the warp threads, and oxidizing the dye during such step, and in discharging a further quantity of dye liquor to the reversed threads, and in oxidizing the second application of dye.

11. The method of applying indigo color to yarn which consists in winding the yarn on a hollow beam, applying indigo color to the yarn while on said beam, removing excess liquor from said yarn, unwinding said yarn from said beam, exposing the yarn to the atmosphere to oxidize the indigo, rebeaming the oxidized yarn, re-dyeing the yarn while rebeamed, unwinding said yarn, exposing the yarn to the atmosphere to oxi-

dize the added color and rebeaming the yarn.

12. The method of applying indigo color to yarn which consists in winding the yarn on a hollow beam, washing the yarn while on said beam, applying indigo color to the 20 yarn while on said beam, removing excess liquor from said yarn, unwinding said yarn from said beam, exposing the yarn to the atmosphere to oxidize the indigo, rebeaming the oxidized yarn, re-dyeing the yarn while 25 rebeamed, unwinding said yarn, exposing the yarn to the atmosphere to oxidize the added color and rebeaming the yarn.

EDWARD T. GARSED.